

Aug. 11, 1931.

J. S. BUSCH

1,818,039

PROCESS OF TREATING FIBROUS MATERIAL PRELIMINARY TO MAKING PULP

Filed Dec. 31, 1928



Inventor:  
John S. Busch.  
By Whitley and Ruckman  
Attorneys.

## UNITED STATES PATENT OFFICE

JOHN S. BUSCH, OF CLOQUET, MINNESOTA

## PROCESS OF TREATING FIBROUS MATERIAL PRELIMINARY TO MAKING PULP

Application filed December 31, 1928. Serial No. 329,505.

My invention relates to processes of treating fibrous material preliminary to making pulp. In carrying out my process, wood or other material containing cellulose preferably in the form of chips or small pieces is subjected to mechanical pressure while submerged in water or other liquid. The term "chips" will subsequently be employed and is to be considered as including small pieces. The pressure which I employ is sufficient to compress and at least partly crush the material and force out some of the air and moisture which it contains. When the pressure is released the tendency of the material is to expand and resume its former shape and this causes some of the liquid surrounding it to be absorbed or soaked up. By successively applying and releasing the pressure, most of the air and moisture originally in the chips are removed and replaced by the liquid in which the crushing operation takes place. After the initial crushing, the amount of liquid forced out of the material by each successive crushing becomes greater and its removal causes the chips to burst, thereby producing partial separation of the fibers. When thus treated, the chips are in excellent condition to be reduced to a pulp by any of the standard types of pulping apparatus. It has been found that the use of hot water or chemicals such as caustic soda and "lignin dissolving" solutions as the liquid in which the crushing operation is performed, greatly hastens the separation of the fibers. In practice it has been found that the crushing can be readily accomplished by means of crushing rolls and that about five successive crushings will give the desired result. It is obvious that other means of applying mechanical crushing upon the chips while immersed in the liquid may be employed. I am aware of the fact that it has been proposed to grind chips while subjecting them to a small stream of water and that it has also been proposed to pass pulp between rollers in a vat containing a solution, but so far as I am aware, it has never before been proposed to subject the chips to crushing action while submerged under a liquid prior to the pulping operation.

The full objects and advantages of my in-

vention will appear in connection with the detailed description thereof, and the novel features of my inventive idea will be particularly pointed out in the claims.

In the accompanying drawing, Fig. 1 is a vertical sectional view of an apparatus suitable for carrying out my process.

Referring to the construction shown in the drawing, the numeral 10 designates a receptacle in the upper portion of which there are two cooperating crushing rolls 12 and 14. A hopper 16 at the top of the receptacle 10 is arranged to deliver chips of the material to be treated between the crushing rolls 12 and 14. The receptacle 10 has a reduced downward extension 18 containing an upper pair of crushing rolls 20 and 22 and a lower pair of crushing rolls 24 and 26. An upwardly inclined casing 28 extends from the bottom of the extension 18. At the upper end of this casing, there is roller 30 while beyond the lower end of the casing and located in the extension 18 there is a roller 32. An endless conveyor 34 is trained around the rollers 30 and 32, the lower stretch of this conveyor passing underneath a curved guide 36, while the upper stretch of the conveyor passes underneath a curved guide 38 so that the lower portion of the conveyor extends horizontally. The conveyor is provided with a plurality of cross pieces 40 which engage the material and move it upwardly. The upper end of the conveyor 34 delivers upon a horizontal conveyor 42 which takes the material to any desired place.

When the apparatus above described is employed for carrying out the process, chips of the material to be treated are fed by the hopper 16 and drop between the rolls 12 and 14 so that the material is crushed below the liquid level in the receptacle 10, it being noted that the level of the liquid is above the axes of the rolls. Ordinarily it will be found that most of the chips will float after one crushing and some of them even after two or three crushings. The floating chips will accumulate at the top of the liquid as indicated at 44 and 46 and will be carried around again between the rolls 12 and 14 until they sink in the liquid. The chips then pass be-

tween the pair of rolls 20, 22, and the pair of rolls 24, 26, and are removed by the conveyor for subsequent treatment to reduce them to pulp. My process produces a softened chip in which the separation of the individual fibers composing the chip has partially taken place. Subsequent treatment of this material in any of the standard disintegrating or pulping machines is accomplished with a greatly reduced power consumption and with the production of a longer and stronger fiber. By performing the crushing operation under hot water, it is found that the cementing materials of the fibers in the chips are considerably softened, thus making a much easier subsequent separation. By the use of chemicals such as solution of caustic soda as the submerging liquid, the resins are dissolved in resinous woods, thus facilitating the subsequent disintegration of the chips. My inventive idea may be employed for impregnating wood chips with chemical solutions by mechanical means, and may be utilized in producing a semi-mechanical and chemical pulp. By performing the crushing operation in a "lignin dissolving" liquid or solution, the lignin can be removed from the chips in whole or in part to produce a semi-chemical pulp. In the use of caustic soda solution, it has been found that the use of temperatures above 212° F. greatly hastens the dissolving of the lignin. In order to accomplish this result, the chips impregnated with the caustic soda solution by the crushing operation may be drained, placed in a digester and subjected to steaming under pressure for a suitable period of time and at a suitable pressure after which they are dumped, washed and disintegrated. The liquors used in the sulphate and sulphite pulping process may also be satisfactorily employed. My process provides a method of treating various woods which cannot be successfully utilized in connection with the mechanical and chemical processes now in use for making pulp. It has been found to be successful in preparing chips of pine, cedar, balm-of-Gilead, poplar, tamarack, and spruce so that such material can subsequently be defiberized by standard mechanical machines with much less difficulty and with decreased power consumption. The process is adaptable for use with other woods and with other material, such as straw, be-gasse, and bamboo.

55 I claim:

1. The process of treating fibrous material preliminary to making pulp which consists in providing chips of the material, feeding said chips downwardly between a pair of horizontal crushing rolls which are submerged for more than half their diameter in a liquid, and repeating the crushing action of the rolls by flotation and inward movement of the chips toward the space be-

tween the rolls until the chips sink in the liquid.

2. The process of treating fibrous material preliminary to making pulp which consists in providing chips of the material, feeding said chips downwardly between a pair of horizontal crushing rolls which are submerged for more than half their diameter in a "lignin dissolving" liquid, and repeating the crushing action of the rolls by flotation and inward movement of the chips toward the space between the rolls until the chips sink in the liquid.

In testimony whereof I hereunto affix my signature.

JOHN S. BUSCH.